

March 31, 1931.

C. BATCHELLER

1,798,998

SHINGLE AND COLORATION THEREOF

Filed June 21, 1926

*Fig. 1.*



*Fig. 2.*



Inventor

CLEMENTS BATCHELLER  
By his Attorneys

*John A. Brown*

## UNITED STATES PATENT OFFICE

CLEMENTS BATCHELLER, OF BROOKLYN, NEW YORK, ASSIGNOR, BY MESNE ASSIGNMENTS, TO BEMIS INDUSTRIES, INC., OF BOSTON, MASSACHUSETTS, A CORPORATION OF DELAWARE

## SHINGLE AND COLORATION THEREOF

Application filed June 21, 1926. Serial No. 117,510.

My invention relates to shingles and coloration thereof, and particularly to composition shingles of the fiber cement type. The object of my invention is to provide a shingle having certain improved characteristics (1) in structure, (2) chemical composition, and (3) appearance. As to the two last mentioned features of novelty, it is to a certain extent related to the subject matter of my copending application Ser. No. 90,157, filed February 23, 1926, over which it presents certain features of novelty and improvement. In its physical characteristics it is a departure.

15 A practical embodiment of my invention is illustrated in the accompanying drawing, in which

Fig. 1 is a perspective view of a shingle disclosing the structural characteristics which 20 embody the invention in one form; and

Fig. 2 is a cross section.

In my application above mentioned I have described an asbestos shingle which is manufactured, in accordance with present methods, to form a laminated product of uniform thickness, is subjected to very heavy pressure, and in the finished product presents smooth, hard faces, the shingle being subsequently treated in accordance with the 25 process there disclosed to impart the desired color effects thereto. A shingle of that type, in spite of its desirable coloration, is objectionably "flat" and inartistic. A greatly improved product from the artistic standpoint 30 results from the practice of my present invention.

Instead of forming the fluid suspension necessary to the manufacture of the laminated product above referred to, I prepare a 40 "mud" mixture of hydraulic cement and fiber (asbestos, for example, although other suitable fiber may be used), and subject the same to a molding operation, preferably effected in a heavy press, the press dies being of such 45 form that a heavy butt or wedge-shaped shingle is produced. The mixture is not only less fluid, but the composition of the solids varies from that of the standard product disclosed in my prior application, in that the 50 proportion of fiber to the hydraulic cement is

increased and is preferably within the range of 15% to 35% fiber to 65% to 85% cement. Preferably the fiber constitutes approximately 25% by volume of the solids of the mixture. Moreover, instead of using the very 55 finely shredded fibers which are mentioned in my prior application, and are common in standard asbestos shingles, I now utilize a coarse fiber. Various grades of coarse fiber may be utilized, but I have found by experience that for my purposes a fiber, say 1/64" to 1/8" in diameter and 1/2" to 3/4" long is best suited to produce the desired results.

After the plastic fiber-cement mass has been molded to shape, the face of the shingle 60 which is to be exposed in use is subjected to the action of a suitable roughing tool, such as a metal brush or the like, which is applied before the initial "set" of the mass. This has the effect of raking up on the surface the 65 coarse fibers, so that they, with a certain portion of adherent cement, stand out from the body of the shingles. Preferably this roughing action is confined to the portion of the 70 surface extending from the butt end 10 of the shingle to, or only slightly beyond, the area 11 which is overlapped by the super-adjacent shingle in use. In this manner 75 the flat back of the super-adjacent shingle lies snugly against the smooth face of the 80 area 11 and thus affords a snug joint between the shingles and reduces the danger of the entry of moisture, and more particularly the effort of wind, which otherwise 85 would tend to pry up the shingles. Approximately at the lower margin of the smooth area 11 of the shingle face, nail holes 12 are formed through the shingle, while the material is still in plastic condition.

A shingle of this construction, even if uncolored, presents a markedly improved appearance since the roughening-up of the surface and the projecting fibers changes the color effect by reason of the resulting lights and shadows.

In order to further increase the attractiveness of the shingle, I color it by the deposit of metallic hydroxides which are bound into the surface. For example, I may subject the shingle or its eventually exposed face, to the 100

action of certain metallic salts which react with the free lime which is either present in the hydraulic cement or added thereto, when the latter is deficient, before the plastic mixture is formed. Thus, when the shingles have set sufficiently so that they can be handled they may be subjected to the action of a suitable metallic salt solution.

The salt solution which may be used may vary widely, and the choice largely depends upon the color desired in the finished product. In any event, the salt must be such that it will react with the lime present to form either an insoluble metallic hydroxide or an insoluble basic salt. The asbestos fibers which are raised from the surface-roughening operation may contain some lime, but the effect of the salt treatment upon the fibers is to produce a coloration of the latter different from the coloration of the shingle body. A variegated tone effect is thus produced which is very artistic and cannot be obtained by following the processes heretofore suggested by me or others.

Of the salts mentioned, most of the so-called heavy metals are applicable, and these have been disclosed in my prior application above mentioned. I have found in application to this new type of shingle that a solution of a copper salt gives particularly satisfactory results. The shingle which has not finally set, but has sufficiently hardened to allow handling, may be immersed in a 20% solution of copper chloride or other copper salt, or copper potassium chloride. I prefer to use the copper chloride, or other salt, which upon reaction will give a soluble lime salt, in order that the color deadening effect of an insoluble calcium salt, such as calcium sulphate, will not lessen the full color otherwise obtained. The shingle is immersed for a period, depending upon the depth or shade of color desired. I have found that immersion for one half hour will give a particularly satisfactory multi-color effect. Where the salt has reacted with the lime, copper hydroxide has been formed, which in turn changes in the air to form the dark colored—black or brownish black—copper oxide.

Where the salt has been absorbed by the fiber, but has not undergone any noticeable reaction, the characteristic greenish blue color of the copper salts is to be found. The exact reaction on the asbestos is not fully understood, but it is a fact that after drying, the copper salt cannot be removed from the asbestos by washing. This may be due to the fixation of the copper salt by means of carbon dioxide of the air, but as pointed out above, the exact chemical phenomenon has not been ascertained.

The treatment which I have just described is appropriate for a shingle in which the preliminary "set" has taken place, and from which the moisture has evaporated at the

shingle surface incident to a couple of days exposure in the air. Where the shingle has been thoroughly dried out, as will occur in the course of a couple of months of aging, it is possible that a briefer immersion in the copper salt solution will suffice by reason of its more rapid penetration into the interior of the shingle. The depth of penetration of the solution will depend upon two factors—first, the period of immersion, and second, the dryness of the article.

I have referred to the possibility that the copper salt which has been absorbed by the asbestos has been made insoluble by the absorption of carbon dioxide from the air, thus forming copper carbonate. This same fixing can be obtained by a subsequent immersion of the shingle treated with the copper salt solution into a warm solution of a soluble carbonate, such as sodium carbonate, whereupon the copper carbonate is bound in and upon the surface of the shingle. If the shingle is immediately immersed in the sodium carbonate solution after treatment with the copper salt solution, and before the copper hydroxide has been changed to copper oxide, practically the entire surface of the shingle will be converted into the copper carbonate, which is a fairly brilliant greenish blue, known to the trade as "mineral green", and substantially permanent. A very beautiful aged copper effect is obtained.

Obviously the same chemical reactions, and the same color effects may be obtained upon the surface of other objects containing free lime, nor is this novel treatment to be limited to the treatment of a shingle whose surface has been roughened, as hereinbefore described; it is equally applicable to a smooth shingle.

I have described shingles which have a multi-colored effect of brownish black and green, and of shingles which are substantially greenish blue in effective color. I have found that if the shingle which has been treated with the copper salt solution is subsequently immersed in a solution of ferro-sulphate, that a mottled green and brown shingle is obtained. The exact relation of one color to the other depends upon the length of time of immersion in the ferro-sulphate, and upon the concentration of the ferro-sulphate. If a shingle is desired in which the green coloration predominates, an immersion in a 10% solution of ferro-sulphate for a few seconds will be sufficient to give a brown or greenish brown tinge at places on the surface.

The chemically untreated shingle may to advantage be immersed in a 20% solution containing three parts by weight of copper chloride, and one part by weight of ferro-sulphate. In this case the two metallic salt solutions simultaneously react with the lime, giving a very desirable greenish brown to brown effect. The depth of the color, as in

the previous examples, will depend upon the length of time of immersion.

While in these specific examples I have stressed the copper and iron salts, it will be obvious that other color effects may be obtained by choosing the salts whose hydroxides are of the desired shade. For example, in place of copper and iron salts, nickel, cobalt or chromium might be used. These variations will be within the skill of one familiar with the color of the metallic hydroxides.

I claim—

1. As a new article of manufacture, a shingle comprising a mixture of cement and fibers, and having a surface roughened by projecting fibers, said roughened surface being colored by an insoluble deposit resulting from the reaction of a metallic salt and the alkaline material of the shingle bound therein.

2. As a new article of manufacture, a shingle comprising a mixture of cement and fibers and having a surface roughened by projecting fibers, said roughened surface being colored by an insoluble deposit resulting from the reaction of a metallic salt and the alkaline material of the shingle bound therein and differing in coloration from the fibers projecting from said surface.

3. As a new article of manufacture, a shingle comprising an alkaline base and fibres and having a surface roughened by projecting fibres, said roughened surface being, surface colored by an insoluble metallic carbonate deposit.

4. The method of coloring a body having a surface roughened by projecting fibres and an alkaline reaction which comprises applying thereto a metallic salt solution which reacts with the alkali to form an insoluble metallic hydroxide deposit and converting the hydroxide into a substantially permanent carbonate.

5. The method of coloring a body having a surface roughened by projecting fibres and an alkaline reaction which comprises applying thereto a copper salt solution which reacts with the alkali to form an insoluble hydroxide of copper, and converting said hydroxide into a substantially permanent carbonate.

6. The method of coloring a body having a surface roughened by projecting fibres and an alkaline reaction which comprises applying thereto a metallic salt which reacts with the alkaline material to form an insoluble colored deposit whereby the roughened surface is colored by the deposit bound therein and is of a different coloration from that of the fibres projecting from said surface.

In testimony whereof I have signed my name to this specification.

CLEMENTS BATCHELLER.